

# UNITED STATES PATENT OFFICE.

STEPHEN M. ALLEN, OF DUXBURY, MASSACHUSETTS.

## MANUFACTURE OF PAPER-PULP, &c.

SPECIFICATION forming part of Letters Patent No. 253,656, dated February 14, 1882.

Application filed August 30, 1881. (No specimens.)

*To all whom it may concern:*

Be it known that I, STEPHEN M. ALLEN, of Duxbury, in the county of Plymouth and State of Massachusetts, have invented a new and 5 useful Improvement in the Manufacture of Paper-Pulp and Leather-Board from Bark and other Wood Fiber, which improvement is fully set forth in the following specification.

This invention has for its object, namely, the 10 production of paper-board or leather-board, although it is in part applicable to other purposes.

It relates to an improved process for making pulp from the fibrous parts of bark of trees, to the combination of bark pulp with 15 other wood fiber, and to an improved leather-board from wood fiber, and process of making the same.

In order to prepare bark pulp in accordance 20 with this invention, the bark is separated from the tree-trunks in sheets, usually first steaming or soaking the wood cut into strips of suitable length to make it come off more easily. The process described in Patent No. 229,307, granted to Jas. Davy, Jr., June 29, 1880, may 25 be employed to advantage. By means of proper sharp cutters the bark can be removed alone, or with a layer of the new wood just below. This new wood I have found can be fibrilized more readily than the part near the 30 heart, and yields a very strong tough fiber. The sheets of bark, with or without the adhering layer of solid wood, are flattened between rollers and fed on a traveling apron or otherwise to a revolving cutter or picker, which is 35 properly gaged to remove the outer or refuse bark, which possesses no valuable fiber, and leave the inner rind or fibers cleaned and perfect. A machine like a common planing-machine with a plain revolving knife or with a 40 toothed cutter, and provided with means such as ordinarily employed for regulating the amount of material taken off, will answer the purpose. The inner bark is then put through a picker which tears it into shreds, is treated 45 with hot water or alkaline solution, and beaten into pulp. It may also be pulped in other ways, although the way described is deemed most advantageous. If it is to be mixed with other fiber or with rag pulp, these can be ground 50 simultaneously with it in the machine forming the subject of my application for patent filed August 15, 1881, for improvement in the manu-

facture of paper-pulp from wood and other materials.

It may be here observed that the manufacture of paper-pulp from bark has been heretofore suggested. It has, for example, been proposed to grind the whole bark and to separate the fibrous from the non-fibrous portions by washing or sifting. None, however, of the 55 processes proposed contemplate the removal of the bark in sheets, nor the separation of the rough and useless bark in the manner indicated; nor do they cover the specific process of making pulp as stated above. In using this 60 pulp it is always preferred to mix it with other fiber, although it can be made into paper or board by itself. It can be subjected to bleaching 65 processes, if desired.

In order to make leather or paper board in 70 accordance with this invention in the most advantageous manner, bark and solid wood are ground together in any suitable machine. The mixed pulp, which should contain about one-third bark and two-thirds solid-wood fiber from 75 new wood or old wood, or both, is placed in a beating-engine wherein it can be heated. While hot it is thoroughly incorporated with asphalt sizing. This sizing consists of a base 80 of pure asphalt melted or softened with any mineral, vegetable, or animal oil, or with other resinous material, in connection with reduced alkalies mixed in hot water. The sizing is used in the proportion of about five to ten parts to ninety or ninety-five parts of pulp. 85 When the materials are well mixed the pulp is run off onto a board-machine of any usual construction and made into sheets of leather or paper board of the desired dimensions. The sizing not only colors and sizes the leather or 90 paper board, but renders it nearly water-proof. Other coloring-matter or sizing can be introduced into the beating-engine, or they may be introduced into the grinder, if desired. The board can also be embossed or painted, if desired. 95 It is excellently adapted to the manufacture of chair seats and backs, to trunk-coverings, as a substitute for patent-leather in saddles and harness, to cap visors and trimmings, to car-sheathing, machine-beltting, roofing, washers for screw-nuts, &c. Paper-board may be made in the manner indicated with various proportions of solid-wood fiber and bark fiber, of solid-wood fiber alone, or of bark fiber alone. 100

More or less rag fiber or fiber from other paper-stock may also be mixed with the wood fiber.

Instead of grinding the solid wood and bark together, they may be made into pulp separately by grinding or other process, and then mixed in the beating-engine, or the bark, after being torn to pieces in the picker, can be added to the disintegrated or ground wood fiber in said engine.

10. In the separation of the rough useless bark from the fibrous portions the latter may be planed off in the form of shavings, leaving the rough portions.

Having now fully described my said invention and the manner of carrying the same into effect, what I claim is—

15. The method of making pulp from bark by separating the rough from the fibrous portion, tearing the latter into shreds by a picker, soaking, and beating, substantially as described.

20. The method of making bark pulp by removing the bark in sheets, separating the rough bark from the fibrous portions by planing, and then tearing the fibrous portions to shreds in a picker, soaking them, and beating them into pulp, substantially as described.

3. The method of preparing bark pulp or making paper, paper-board, and like articles, by mixing the bark pulp with or without pulp from solid wood or other material, while hot, 30 with asphalt sizing or other sizing, substantially as described.

4. Paper-pulp, paper, paper or leather board, or other manufacture of paper containing bark pulp alone or with other fiber sized with asphalt 35 sizing, substantially as described.

5. The combination in paper-pulp, paper, paper or leather board, and the like, of bark pulp and solid wood pulp, substantially as described.

40. 6. A paper or leather board of bark pulp and solid-wood or other pulp, sized and colored with asphalt sizing, or other sizing and coloring materials, substantially as described.

In testimony whereof I have signed this 45 specification in the presence of two subscribing witnesses.

STEPHEN M. ALLEN.

Witnesses:

H. G. ALLEN,  
C. J. HEDRICK.